

## UNITED STATES PATENT OFFICE

JOHN JOHNSTON, OF SHORT HILLS, NEW JERSEY, ASSIGNOR TO UNITED STATES STEEL CORPORATION, OF NEW YORK, N. Y., A CORPORATION OF NEW JERSEY

## CORROSION RESISTANT CHROMIUM ALLOY MANUFACTURE

No Drawing.

Application filed June 25, 1931. Serial No. 546,921.

This invention relates to metallurgy and more particularly to chromium-containing corrosion resistant alloys and to methods of manufacturing the same.

5 Heretofore in the art it has been customary to comprise chromium-containing corrosion resistant alloys of a relatively high proportion of chromium. It is estimated that it requires more than about 12 percent 10 of chromium in iron, for example, to impart thereto the corrosion resisting properties of the chromium. It is well known that carbon is detrimental to the corrosion resisting properties of such alloys.

15 This has been attributed to the fact that chromium forms a relatively stable chromium carbide compound having the empirical formula  $\text{Cr}_4\text{C}$  in which approximately one molecular weight of carbon combines with 20 approximately four molecular weights of chromium or that each unit weight of carbon present in the alloy combines with about sixteen unit weights of chromium. It is apparent therefore that a relatively small amount 25 of carbon will have a pronounced effect on the chromium content of the alloy. It is difficult to reduce the carbon content of such alloys below approximately 0.06%, and it has been found that even such small amounts 30 of carbon may be detrimental to corrosion 35 resistant chromium alloys when they are subjected during service to elevated temperatures.

It has been proposed to overcome the detrimental effect of this relatively low and unavoidable carbon content of chromium containing corrosion resistant alloys by the addition to the alloy of a proportion of a metal or metals which react with the carbon to 40 form carbide compounds in the alloy structure which are more stable than the chromium carbide compound. This effectively eliminates the carbon from the alloy structure and the deleterious effects thereof are 45 not experienced. Those metals which have been proposed comprise titanium, zirconium, tungsten and molybdenum. Of these titanium has been preferred for economic and practical reasons and also for the reason 50 that the titanium carbide compound formed

does not appear to deleteriously affect the workability of the resulting alloy.

The usual procedure heretofore practiced in the addition of titanium to chromium-containing corrosion resistant alloys is to 55 add the titanium to the fused corrosion resistant alloy mixture employing an excess of titanium to ensure the total conversion of the carbon to the titanium carbide compound. In some cases it has been suggested 60 to use an excess up to 5 to 10% titanium; such an excess of titanium, however, would be largely present as an alloying constituent in the final alloy.

For some purposes it is desirable to obtain 65 a low-carbon chromium-containing corrosion resistant alloy in which there is substantially no excess of titanium present as an alloying constituent and in which the carbon content is comprised substantially of titanium carbide (or its equivalent). Under prior art 70 methods of forming titanium containing alloys, this is not practical.

It is one of the objects of the present invention to obtain such an alloy product. 75

It is another object of this invention to provide a method of manufacturing such an alloy.

It is another object of this invention to improve the method of manufacturing chromium-containing corrosion resistant alloys. 80

Still another object of this invention is to provide a method of introducing relatively small amounts of a highly reactive constituent 85 into chromium-containing alloys.

Other objects and advantages will become apparent as the invention is more fully disclosed.

In accordance with the objects of my invention I have found that a large part of the carbon in chromium-containing corrosion resistant alloys is incorporated therein as a constituent of the ferro chromium alloy utilized in the compounding of the same. It is difficult to obtain a substantially carbon-free ferro chromium alloy which does not also contain deleterious amounts of aluminum, silicon and the like metalloids. 95

I have found, however, that if the carbon containing ferro chromium is first admixed 100

with titanium (or its equivalent) in such manner as to convert all or substantially all of the carbon content thereof to titanium carbide, the resultant ferro chromium alloy 5 product may be utilized in the forming of corrosion resisting chromium alloys free from the accompanying detrimental carbon effects. I have also found that by providing an excess of titanium in the ferro chromium this 10 excess may be subsequently utilized as a carbon fixing agent for the residual carbon in the metal comprising the base for the corrosion resistant alloy product without the undue losses heretofore experienced and without using a relatively large excess of the 15 titanium as has heretofore been necessary. This is believed due to the fact that the usual residual carbon of the alloy base to which the chromium is added is more readily converted to titanium carbide than is chromium carbide.

By control analyses and by proper calculation, the total carbon content of the corrosion 20 resistant alloy may be readily determined and the amount of titanium added thereto as a constituent of the ferro chromium alloy readily controlled. It is apparent that I may use the titanium containing ferro chromium alone in the forming of the corrosion 25 resistant alloy, or I may utilize it in part admixed with low carbon ferro chromium, if desired. It is preferable, however, to utilize the titanium containing ferro chromium alone 30 as the chromium carbide content thereof has been substantially reduced or converted over 35 into the desired inert stable titanium carbide compound prior to addition to the corrosion resistant alloy base.

It is not contemplated as within the scope 40 of the present invention that the titanium, or its equivalent, will be present in the resultant corrosion resistant alloy product in amounts substantially greater than is necessary to react with and combine with the total carbon 45 content of the alloy to form a stable metal carbide compound. Stoichiometrically, the amount of the titanium necessary would be approximately four times the amount of the total carbon content of the alloy, but owing 50 to the fact that the carbon content of the alloy base is in a greatly diluted form, it is necessary to add a somewhat greater amount of titanium. I have found that in general 55 the amount of titanium added should approximate from 6 to 8 times the total carbon present. Amounts in excess of this may be construed as being an alloying constituent and for the purposes of this invention 60 undesirable.

The chromium-containing corrosion resistant alloy products of the present invention may be comprised of iron base alloys or of the iron nickel base alloys and may be comprised in part of other alloying constituents 65

such as manganese, silicon, aluminum, copper, cobalt and the like.

As a specific embodiment of the practice of the present invention, I will disclose the same as it may be utilized for the preparation of the well known so-called 18-8 type of chromium-nickel-iron alloy containing approximately 18% chromium, 8% nickel less than 0.1% carbon and the balance mainly iron. I 70 prepare the titanium containing low carbon ferro chromium either by melting up low carbon ferro chromium and adding the proper proportion either of titanium or of a mixture of titanium oxide and reducing agent which by reaction yield titanium; or I can mix a titanium ore, such as rutile or ilmenite, or a titaniferous iron ore, each in proper proportion, with the chrome ore from which the ferro chromium is made. The desired chromium nickel iron alloy is then made by adding this modified ferro chromium in the usual way in amount sufficient to yield the desired chromium content, to a melted bath of low carbon steel to which the proper amount of nickel has been added. I may employ the 75 titanium containing ferro chromium in order to reach to proper final content of titanium. This is adjusted on the basis of the total carbon present in the fused alloy so as to be sufficient to combine with the total carbon to form 80 a titanium carbide compound. The titanium should be preferably added in sufficient excess to allow for such losses as may be due to interaction with oxides, nitrides and the like components of the steel bath but not in sufficient amounts as to become thereby an alloying constituent of the steel. An amount in excess of approximately 6-8 times the carbon content of the steel should be avoided.

Preferably I adjust the components of the final alloy as closely as possible to the desired composition with respect to chromium and nickel, maintaining carbon less than 0.1% (but preferably approximately 0.06%), and the titanium at least in the proportion of approximately four times the weight of the carbon, but preferably from 6 to 8 times the carbon, and the balance mainly iron. Residual amounts of impurities of manganese, silicon, aluminum, phosphorus and sulphur are usually present. Manganese or copper may be substituted in part for the nickel, and other alloy constituents such as vanadium and cobalt, for example, may be present in various amounts, if desired. The silicon content may be increased beyond the normal residual ranges but the phosphorus and sulphur impurities should be substantially eliminated.

Having with particularity broadly and 125 specifically disclosed the present invention, it is believed apparent that there may be many modifications and departures made from the specific embodiment disclosed herein without departing essentially from the na- 130

ture and scope of the invention as may be set forth in the following claims.

What is claimed:

- 5 1. In the manufacture of corrosion resisting chromium steels, the method of incorporating titanium therein which comprises adding the same as a low carbon iron-chromium-titanium alloy, the titanium content thereof being in excess of that amount necessary to empirically combine with all of the carbon content thereof.
- 10 2. In the manufacture of corrosion resisting chromium-nickel steels, the method of incorporating titanium therein which comprises adding the same as an iron-chromium-titanium alloy having a low carbon content and a titanium content at least ranging from

six to eight times the said carbon content.

3. In the manufacture of low carbon corrosion resisting chromium-nickel steels, the method of effectively eliminating the carbon therefrom which comprises incorporating therein a proportion of a low carbon iron-chromium-titanium alloy, the titanium content thereof being in excess of that necessary to empirically combine with the said carbon, the proportion of said alloy added being at least sufficient to bring the titanium content of the steel to about six to eight times the total carbon of said steel.

In witness whereof, I have hereunto signed my name.

JOHN JOHNSTON.

20

85

25

90

30

95

35

100

40

105

45

110

50

115

55

120

60

125

65

130